

July 16, 1929.

J. H. YOUNG

1,720,708

BUILDING MATERIAL

Filed April 6, 1922

Fig. 1.



Fig. 2.



Fig. 3.



Inventor.  
James Howard Young  
Att.  
Jas. H. Churchill  
Atty.

## UNITED STATES PATENT OFFICE.

JAMES HOWARD YOUNG, OF PITTSBURGH, PENNSYLVANIA, ASSIGNOR TO H. H. ROBERTSON COMPANY, OF PITTSBURGH, PENNSYLVANIA, A CORPORATION OF PENNSYLVANIA.

## BUILDING MATERIAL.

Application filed April 6, 1922. Serial No. 550,226.

This invention relates to building material and particularly shingles and has for its object to provide a relatively rigid shingle which has the desirable fire and weather resisting properties and also the artistic value of a copper shingle and which can be produced at a materially less cost.

To this end, the shingle is provided with a relatively rigid foundation member composed of a mixture of cement and fibrous material, such as asbestos, mineral wool and the like, and said foundation member has affixed to it a relatively thin layer of metal, preferably one of the so-called non-corrodible metals, such as zinc, lead or the like, which metal in a molten state is projected or sprayed in a finely divided condition onto the rigid foundation member, so that the metal particles are welded or molecularly united together to form the relatively thin metal layer, upon which is deposited a relatively thin layer of copper. The copper layer may be deposited by electrolysis or by dipping the sprayed metal layer into solutions of the proper copper salts.

The copper layer is capable of being colored by known chemical means to give desirable color effects, such as green, blue or brown, and thereby produce a shingle of high artistic value.

These and other features of the invention will be pointed out in the claims at the end of this specification.

Fig. 1 is a plan view with parts broken away of a shingle embodying this invention.

Fig. 2, a cross section on an enlarged scale of the shingle shown in Fig. 1, the section being taken on the line 2-2, and

Fig. 3, a cross section of a modified form of shingle.

Referring to the drawing, *a* represents the foundation member of the improved building material which is herein represented as a shingle.

The foundation member *a* is relatively rigid and composed of a mixture of cement 10 and asbestos or other fibrous material 12, which in itself possesses certain fire and weather resisting value, which is materially increased by providing the foundation member with a relatively thin layer *b* of metal, preferably zinc, lead or the like so-called non-corrodible metals.

The layer *b* is affixed to the foundation

member by spraying or projecting molten 55 zinc, lead or like metal by means of fluid pressure, upon the foundation member *a* so as to completely cover the same as represented in Fig. 2, or to partially cover the same as represented in Fig. 3. The layer *b* 60 thus applied comprises individual metal particles fused or welded together to form a continuous coating while retaining the irregular contour of the individual particles as illustrated in Figs. 1, 2 and 3 of the drawing. 65

The finely divided particles of the molten metal projected upon the foundation member are welded together or molecularly united to form the relatively thin metal layer *b*, upon which a layer *c* of copper is deposited. 70 The copper layer *c* may be deposited by the well known electroplating methods or by dipping the metal layer *b* into solutions of the proper copper salts, such for instance as

The deposited copper layer *c* firmly adheres to the sprayed metal layer *b*, and adds materially to the fire and weather-resisting value of the foundation member *a* and the metal layer *b*, and in addition imparts to the shingle high artistic values, inasmuch as the 80 copper layer *c* can be colored by known chemical means, to give desirable color effects, such as green, blue or brown.

The metal layer *b* may be formed by air or other fluid pressure after the manner represented in U. S. Patent No. 495,107 dated April 11, 1893.

The shingle herein represented is of substantial thickness and when erected upon the building has the appearance of a solid copper 90 shingle.

The cement shingles which are in use are non-hygroscopic. Otherwise they would not have a value of being unaffected by climatic or weather conditions, nor would they have 95 a value of being heat resistant and fireproof. Because of the use of cement, which before hardening is plastic, they may be molded and when hardened they do not warp or expand detrimentally. Because of the fact that the cement shingles are molded, natural irregularities occur, and because of the fact that either or both metallic coatings are thin and because of the method of application to the cement shingle, either or both coatings 100 will conform to the irregularities. The purpose of my invention is to improve upon this type of shingle as hereinbefore pointed out.

I have herein described the building material as a shingle, but it is not desired to limit the invention in this respect.

I claim:

- 5 1. An improved building material having a foundation member of cement and fibrous material, a relatively thin non-corrodible metal layer affixed to said foundation member and comprising individual metal particles fused together to form a continuous coating while retaining the irregular contour of the individual particles, and a relatively thin layer of copper bonded to said first-mentioned metal layer.
- 10 2. An improved building material having a foundation member of cement and asbestos fibre, a relatively thin non-corrodible metal layer affixed to said foundation member and comprising individual metal particles fused together to form a continuous coating while retaining the irregular contour of the individual particles, and a relatively thin layer of copper bonded to said first-mentioned metal layer.
- 15 3. An improved building material having a relatively thick rigid foundation member of non-metallic material, a relatively thin metal layer affixed to said foundation member and comprising individual metal particles fused together to form a continuous coating while retaining the irregular contour of the individual particles, and a relatively thin layer of copper bonded to said first-mentioned metal layer.
- 20 4. An improved shingle having a foundation member of cement and asbestos, and a relatively thin non-corrodible metal layer affixed to said foundation member and comprising individual metal particles fused together to form a continuous coating while retaining the irregular contour of the individual particles, and a relatively thin layer of copper bonded to said first-mentioned metal layer.
- 25 5. An improved shingle having a foundation member of cement and asbestos, and a relatively thin non-corrodible metal layer affixed to said foundation member and comprising individual metal particles fused together to form a continuous coating while retaining the irregular contour of the individual particles.

In testimony whereof, I have signed my name to this specification.

JAMES HOWARD YOUNG.